

Sept. 19, 1939.

C. F. HERINGTON

2,173,586

TWIN ANNEALING OVEN

Filed Nov. 18, 1936

5 Sheets-Sheet 1



Sept. 19, 1939.

C. F. HERINGTON

2,173,586

TWIN ANNEALING OVEN

Filed Nov. 18, 1936

5 Sheets-Sheet 2



INVENTOR  
Cecil F. Herington  
by William B. Jeppson  
Attorney.

Sept. 19, 1939.

C. F. HERINGTON

2,173,586

TWIN ANNEALING OVEN

Filed Nov. 18, 1936

5 Sheets-Sheet 3



INVENTOR  
Cecil F. Herington  
by William B. Jasper  
Attorney.

Sept. 19, 1939.

C. F. HERINGTON

2,173,586

TWIN ANNEALING OVEN

Filed Nov. 18, 1936

5 Sheets-Sheet 4



INVENTOR  
*Cecil F. Herington*  
by *William B. Jasper*  
*Attorney.*

Sept. 19, 1939.

C. F. HERINGTON

2,173,586

### TWIN ANNEALING OVEN

Filed Nov. 18, 1936

5 Sheets-Sheet 5



Fig. 6.

Fig. 7.

**INVENTOR**

INVENTOR  
Cecil F. Herrington  
by William B. Jasper  
Attorney.

## UNITED STATES PATENT OFFICE

2,173,586

## TWIN ANNEALING OVEN

Cecil F. Herington, Bellevue, Pa., assignor to  
Amco, Incorporated, Pittsburgh, Pa., a corpora-  
tion of Pennsylvania

Application November 18, 1936, Serial No. 111,369

2 Claims. (Cl. 263—28)

This invention relates to new and useful improvements in apparatus and method of annealing castings, and it is among the objects thereof to obtain a relatively short annealing cycle in the production of malleable iron with the advantages of prompt shipments, reduction in inventories, saving in equipment and increased production capacity of the annealing equipment.

That the reduction of the malleableizing cycle may be accomplished through better furnace design and atmosphere control to reduce the time for bringing the charge to heat and for cooling, and by the elimination of use of packing materials has been generally recognized, but seemingly

15 ignored in commercial practice.

In accordance with the present invention, a short annealing cycle for malleable iron is attainable by a twin annealing oven unit, one of which is operated at greater temperature than 20 the other, and both of which are fired from a common heating source, thereby conserving heat and fuel. By transferring the charge from one of the twin oven units to the other without necessitating cooling of the high temperature furnace 25 to the lower temperature desired, the annealing capacity of such furnace is greatly increased and there is little or no time lost in generating the necessary temperature condition in either of the twin oven units.

30 The invention further contemplates the provision of a system of transfer cars and tracks to facilitate handling of the charges in and around the furnaces.

A commercial form of apparatus for reducing 35 the malleableizing cycle in accordance with the above stated objects is shown in the accompanying drawings constituting a part hereof in which:

Fig. 1 is a half front elevational and half-cross sectional view of a furnace unit embodying the 40 principles of this invention;

Fig. 2 is a horizontal cross-section of the high temperature furnace taken along the line 2—2, Fig. 1;

Fig. 3 a horizontal cross-sectional view of the 45 low temperature furnace;

Fig. 4 a longitudinal vertical cross-sectional view of the high temperature furnace shown in Fig. 2;

50 Fig. 5 a longitudinal vertical cross-sectional view of the low temperature furnace shown in Fig. 3;

Fig. 6 a diagram illustrating the annealing cycle; and

55 Fig. 7 a diagrammatic view of a factory lay-

out showing the arrangement of furnace and track.

While the apparatus shown in the drawings is suitable for annealing in malleable iron or steel foundry practice, the temperature figures herein-after referred to as illustrating an embodiment 5 of the invention are the annealing temperatures for malleable iron.

With reference to Fig. 1 of the drawings, the furnace unit comprises a suitable base or foundation 1 of concrete upon which is mounted a pair of rails 2 for supporting a truck 3 constituting the furnace hearth, the truck being mounted on wheeled axles 4 which traverse the rails 2 and the sides of the trucks are provided with a depending flange 5 carrying sand 6, which seals the upper furnace chamber by engagement with a depending flange element 7.

The furnace chamber is constituted by arched side walls and a roof 9 as shown in the half cross section, which constitutes a muffle chamber heated by the products of combustion which are produced by a gaseous flame introduced through a series of firing ports 10 at the sides of the furnace adjacent the top thereof, and a roof structure 11 forming a heating chamber with the roof tile 9 of the muffle into which the products of combustion are delivered. A series of vertical flues 12 constitutes waste gas passages for the products of combustion which are exited through bottom openings 13 in the side walls of the furnace into a waste gas passage 14, dampers 15 being provided to control the distribution of heat longitudinally of the furnace by regulating the volumes of the waste gases withdrawn at any portion of the furnace throughout its longitudinal extent. Control of temperature is also obtainable by the regulation and number of the firing ports 10, of which four are shown in Fig. 2 of the drawings in staggered relation to effect a 40 blanketing of the muffle by a heat flame extending transversely of the muffle wall.

Both the front and rear of the furnace walls are provided with relatively large openings controlled by doors 16 which are suspended and provided with counter-weights 17 to facilitate opening and closing of the furnace doors. The doors are suitably insulated to reduce loss of heat by radiation. The outer furnace wall is reinforced by the usual buck stays 18 and channels 19 to provide a rigid construction and heavy wall insulation 20 is employed to minimize the fuel input to the furnace.

The construction of the lower temperature furnace of Figs. 3 and 5 is similar to the high tem- 55

perature furnace described in connection with Figs. 1, 2 and 4 excepting for the absence of the burner ports 10, the heat being supplied through the waste gas conduits 14 which extend from the high temperature furnace to the low temperature furnace and communicate with the heating chamber of the furnace through the passages 13a and vertical flues 12a. Combustion chambers 21 may be provided in the space intermediate the high and low temperature furnaces to generate the high auxiliary source of heat which is communicated direct to the conduits 14 for delivery to the low temperature furnace through the openings 13a at the bottom of the furnace, the aggregate waste gases of the two furnaces being removed through a stack 22 which is controlled by a damper 23. The conduits 14 are provided with dampers 24 at their respective ends to regulate the air supply to the low temperature furnace as desired.

In the factory lay-out diagram of Fig. 7, the arrangement of furnaces and track is shown to be such that the car supporting the castings is moved from a transfer track into the high temperature oven, thence into the intervening space between the high and low temperature ovens, then to the low temperature oven from which it travels to a transfer track and then a return track to be recharged and again moved through the furnace. The dotted portion of the diagram illustrates an additional installation of a twin furnace unit to provide for increased annealing capacity with economy of space.

In utilizing the above described apparatus for short malleableizing annealing cycles, the castings loaded on the truck 3 are delivered to the furnace of Fig. 2 of the twin annealing oven unit, wherein it is subjected to temperatures of 1700° F. for ordinary malleableizing, although for some malleable foundries, temperatures as low as 1500° F. may be used and 900° F. is the normal temperature at which the furnace is operated for steel castings.

By controlling the fuel delivered through the firing ports 10 and the distribution of the products of combustion by manipulation of dampers 15, a uniform temperature is maintained throughout the furnace chamber, thereby subjecting the charge to uniform heat and the waste gases from the high temperature furnace are withdrawn through passages 13 into the waste gas conduit from which they are conveyed into the furnace shown in Fig. 3 which is operated at a temperature of about 1350° F. or otherwise as desired.

The charge is maintained at a uniform temperature of substantially 1700° F. in the first furnace unit, Fig. 2, for a period of about 24 hours after which the car is removed into the intervening space between the two furnaces, and the charge allowed to cool to a temperature of substantially 1250° F. The car with its charge of castings is then moved into the second furnace shown in Fig. 3 and subjected to the 1350° F. temperature for a period of about twenty-eight hours or as desired. The furnaces are thus continually operated since a new charge is placed into the high temperature furnace immediately when the first charge has been removed.

Very little heat is required to bring the charge up to the critical temperature in the second furnace as the charge and supporting truck is already at a temperature of 1250° F. when they are charged into the second furnace.

If the products of combustion from the high temperature furnace have dropped in temperature below the temperature of 1350° F. required

in the second furnace, additional heat is supplied through the auxiliary combustion chambers 21 and if the temperature of the products of combustion from the first furnace is in excess of that required in the second furnace, the temperature can be reduced by admitting air through the openings of manifolds 14 controlled by the dampers 24.

The production capacity of the twin furnace unit on short cycle annealing is best understood with reference to the diagram of the annealing cycle of Fig. 6 which is for a week of one hundred and sixty-eight hours employing a cycle of sixty-seven hours for each car containing ten to twelve tons of castings. The cycle shows plainly that every thirty-four hours a new load is placed in the first oven and a car removed from the second oven for unloading. This gives an annealing capacity of two hundred tons of castings a month.

The fuel economy obtainable is dependent on the cost of fuel, oil or gas at the point of use, but by the use of the muffle type oven the manner of firing and control of heat application a saving of more than thirty percent over conventional forms of annealing ovens is possible.

Annealing pots are unnecessary, thus requiring less initial investment in equipment and a reduction in the heat absorption of the mass passing through the furnace. If, however, circumstances require the use of pots, they may obviously be employed with a resultant lengthening of the annealing cycle but with less erosive effect on the pots, which will last indefinitely. If the castings to be annealed are of a kind in which oxidation should be prevented, a cover may be provided for the truck or charge when it is moved to the air cooling space between the twin oven unit.

From the foregoing description of the invention, it will be apparent that substantial saving in time and fuel are available over the conventional type of long cycle annealing ovens in which, after firing has been stopped, cooling is accelerated by opening dampers to drop the temperature to the critical point, which ties-up such furnaces for the entire annealing cycle, and requires reheating of a substantial temperature range when recharged for a subsequent annealing of castings.

Although one embodiment of the invention has been herein illustrated and described, it will be apparent to those skilled in the art that various modifications may be made in the details of construction without departing from the principles herein set forth.

I claim:

1. A twin oven unit for annealing castings comprising a pair of heating ovens in tandem having a space therebetween, said ovens having muffle chambers for receiving the charge to be annealed and having outer walls forming a combustion space with the muffle wall, means for introducing a gaseous fuel into the firing chamber of one of said ovens and means for withdrawing the products of combustion through vertical flues at the bottom of said oven, a waste gas conduit for delivering the products of combustion to the second of said ovens, said conduit constituting a manifold having a plurality of passages leading to vertical flues of the second named oven to direct the products of combustion around the muffle of said oven and to a stack at the top of said oven, and means for regulating the distribution of the products of combustion in

said ovens to obtain uniform temperatures throughout the heating chambers.

2. A twin oven annealing unit comprising a pair of ovens in tandem having a track extending therethrough and being spaced apart to permit exposing the charges to the atmosphere in their travel on said track from one to the other of said ovens, trucks movable on said track and constituting a hearth for said ovens transferable from one oven to the other and having seals for prevention of heat loss through the bottom of the ovens, said ovens comprising a muffle wall cooperating with the movable trucks to constitute heating chambers, one of said ovens having

burner ports above the muffle wall, and both ovens having an outer wall and roof structure forming a combustion space having vertical flues extending downwardly on the sides of the ovens provided with dampers for regulating the volume of the gases passing through said flues, and a manifold on the respective sides of said ovens having passages connecting with said flues at the bottom thereof to remove the products of combustion in regulable quantities from the longitudinal extent of one side of one of said ovens and deliver said gases through the manifold passages to the same side on the other of said ovens.

CECIL F. HERINGTON.